

M. E. DUNLAP.  
PROCESS OF COATING WOOD.  
APPLICATION FILED NOV. 5, 1918.

1,329,381.

Patented Feb. 3, 1920.

Fig. 1.



Fig. 2.



Inventor.

Matthew E. Dunlap.

# UNITED STATES PATENT OFFICE.

MATTHEW E. DUNLAP, OF MADISON, WISCONSIN, ASSIGNOR TO UNITED STATES OF AMERICA.

## PROCESS OF COATING WOOD.

1,329,381.

Specification of Letters Patent.

Patented Feb. 3, 1920.

Application filed November 5, 1918. Serial No. 261,210.

To all whom it may concern:

Be it known that I, MATTHEW E. DUNLAP, a citizen of the United States, residing at Madison, in the county of Dane and State 5 of Wisconsin, have invented certain new and useful Improvements in Processes of Coating Wood, of which the following is a specification.

My invention relates to methods or processes of coating or finishing articles and has special reference to such as are applicable to 10 aerial propellers and other devices made of wood.

It is well known that many experiments 15 have been made in an attempt to procure coverings for aerial propellers, but so far these have not proven satisfactory. The coatings or finishings thus far made require an expensive apparatus, as in the case where 20 metal is sprayed, or electrolytically deposited and even these coatings when applied are too heavy, do not adhere well, and are torn loose by centrifugal force when the propellers are in action. Other methods have also been 25 formulated differing in scope from those mentioned above which have not been reliable in regard to the exclusion of moisture.

One object of my invention is to provide 30 a simple and effective process of coating or finishing articles whereby a metallic covering is produced which when applied becomes closely associated and intimately united with the article itself.

Another object of my invention is the 35 provision of the process of coating which shall comprise a combination of definite steps which are adapted to coöperate in the production of a metallic covering possessing many advantages over coatings produced by 40 either or the steps taken alone.

The principal object is to provide a process of coating or finishing articles and especially aerial propellers whereby a coating of metal leaf is applied which will be substantially 45 moisture proof, intimately adhesive, and will constitute a coating which is lighter and cheaper than those hitherto used, and also well able to resist adverse atmospheric conditions.

With these and other objects in view the invention consists in certain novel features which will more fully appear as the descrip-

tion proceeds, the novel features thereof being pointed out in the appended claims.

Referring to the drawings which show the 55 preferred embodiments of my invention:

Figure 1 is a side elevation of a propeller blade to which the coating is applied.

Fig. 2 illustrates the completion of the process with the metal leaf affixed about the 60 varnished surface of the propeller, the additional coat of varnish applied about the metal surface, and the intermediate steps shown therebetween.

As disclosed in the drawing a propeller 65 blade 4 is to be coated with my covering. In the process of coating a filler 5 of the standard type is first applied to the wooden blade and after this step one or more coats of varnish 6, depending on the character of the 70 wood as best shown in Fig. 2, are next affixed. Ample time being allowed for the varnished surface to dry, a sanding process is next begun whereby the varnished surface is sanded until smooth. The operation of the 75 coating as thus far advanced has filled all the pin holes and inequalities in the exposed surface, thus presenting a suitable ground for the application of the metallic covering.

The surface after being sanded is coated 80 with a varnish which is used as a size. This coating 7 is allowed to partially dry until a proper "tack" is reached (by the term "tack" as used here is meant the condition of the surface covered with varnish when it 85 is not too dry to prevent metal leaf being applied thereto.)

Metal leaf or foil 8 such as aluminum or imitation gold, which is employed in this process, as a moisture excluding element and 90 which is the principal ingredient of the improved coating, is now applied to the "tacky" surface. This metal leaf may be applied either in a series of wrappings, or in leaf form.

Approximately six hours after the metal leaf has been applied the metal surface is coated with a liquid composition 9, preferably varnish. It is to be understood, however, that the composition applied thereon is 100 not to be limited to varnish as lacquer or enamel may be successfully employed.

To complete the formation of the moisture proof coating one or more coats of the above

mentioned liquid compositions may be utilized, depending entirely upon the circumstances or desirability of having a thick coat of liquid over the metal leaf.

- 5 5. Practical use has shown that after the coating has been applied it is very difficult to disturb the coating and separate it from the article covered. Exhaustive tests have likewise shown, first, that the metal leaf applied about wooden articles has the ability to resist adverse atmospheric conditions, and second, that the metal leaf is not easily susceptible to corrosive agencies. Experiments have also been made which show that
- 10 15 wood covered with a filler and three coats of spar varnish will take up approximately seventeen grams per square foot of surface, when subjected to a humidity between ninety-five and one hundred per cent., and at 20 a room temperature between seventy-five and eighty degrees Fahrenheit, while under the same conditions the same kind of wood after having been treated in accordance with my invention will take up only approximately 25 four tenths of a gram per square foot of surface.

It is to be understood that this invention is not limited to the treatment of propeller blades, but other materials may be treated 30 in the manner above described within the spirit and scope of my invention as claimed.

What I claim is:

1. The herein described process of treating wood which consists in applying a coat 35 of varnish to the wood to be treated, coat-

ing the entire varnished surface with metal leaf, and applying a coat of varnish to the metal surface.

2. The herein described process of treating wood that consists in applying a coat of 40 moisture repellent liquid to the wood to be treated, coating the entire surface with metal leaf and applying another coat of liquid on the metal surface.

3. The herein described process of treating wood which consists in applying a filler to the wood to be treated to provide a smooth surface, impregnating the surface with a liquid composition, affixing metal leaf about 45 said surface, and lastly applying a coat of 50 liquid to the metal leaf.

4. The herein described process of treating wood which consists in applying a filler to the wood to provide a smooth surface, coating the surface with a liquid composition, sizing the surface, affixing a metal leaf 55 to the surface before the liquid thereon is dried, and then applying a coat of liquid to the metal leaf.

5. The herein described process of treating wood which consists in applying a filler to the wood to provide a smooth surface, coating the surface with varnish, sizing of 60 the surface, affixing metal leaf to said surface to seal the wood against moisture, and 65 applying a coat of varnish to the metal surface.

In testimony whereof I affix my signature.

MATTHEW E. DUNLAP.